

## UNITED STATES PATENT OFFICE

1,979,787

## WAX POLISH

Maurice H. Arveson, Hammond, Ind., assignor to  
Standard Oil Company, Chicago, Ill., a corpora-  
tion of Indiana

No Drawing. Application June 22, 1931,  
Serial No. 546,168

11 Claims. (Cl. 134—24)

This invention relates to a solid wax polish for use on automobiles, furniture, etc.

The object of this invention is to provide a polish which will give a lasting, tough, hard, durable wax coating and which may be applied without the use of an abrasive and without undue manual effort.

There are at present two general types of automobile polishes. One type is applied as a liquid or cream, which contains an abrasive, soap and/or cleaning material in addition to an oil and a soft wax base, and although a single application is sufficient to obtain an oily or waxy coating, the resulting coating is usually soft, shows finger prints and is not lasting. The other type of polish gives a much harder and more permanent type of coating, but it must be preceded by the use of an abrasive cleaner, the cleaner must be thoroughly removed and the application of the wax itself requires a great amount of manual effort. The object of my invention is to obtain the hard, tough, durable coating of the latter without the use of a "cleaner" and with the manual ease which characterizes the use of the former.

In practicing my invention I make a wax base of a hard wax-like carnauba or japan wax and a plasticizing agent such as petroleum or a mixture of petrolatum and petrolatum wax. I heat the wax base above its melting point and incorporate it in an oil-in-water emulsion which is prepared in such a manner that it will "set" or solidify on cooling. The oil is sufficiently non-volatile to act as a carrier to effect distribution of the wax on the surface to be polished and it is sufficiently volatile to be completely evaporated from the surface after a few moments of rubbing. The polish has all the advantages of solid wax polishes and it is in fact a solid cake. At the same time it is an aqueous emulsion and it may therefore be applied to an automobile surface which has not been previously cleaned (of course any abrasive material must be removed which would scratch the surface when the polish is being applied).

My invention will be more clearly understood from a description of my preferred formula and my preferred method of processing the ingredients. I will first describe the preparation of my wax base containing hard wax and plasticizing agent. I will then describe the preparation of

the emulsion and the incorporation of the wax base therein.

The wax base may be made by melting together the following ingredients:

|                                               | Percent by weight |
|-----------------------------------------------|-------------------|
| Carnauba wax                                  | 66.5              |
| Petrolatum wax (160 to 165° F. melting point) | 26.6              |
| Petrolatum (140° F. melting point)            | 6.3               |
| Rosin                                         | 0.6               |

It should be understood, of course, that the above formula is illustrative only and that I may vary somewhat from the above proportions without departing from my invention. Carnauba wax or japan wax are my preferred hard waxes but I may use others, such as candelilla, Montan wax, etc. Petrolatum wax is a tough, amorphous (non-crystallin) oil-free, petroleum wax which resembles beeswax in appearance and physical properties. Ordinary commercial petrolatum is petrolatum wax admixed with a small amount of residual oil. Petrolatums of different melting points may be used in other proportions without departing from my invention. Rosin may, if desired, be omitted entirely.

My finished polish may be made according to the following formula:

|                                      | Percent |
|--------------------------------------|---------|
| Wax base prepared as above described | 80      |
| Refined oil (narrow cut)             | 9       |
| Emulsifier                           | 41      |
| Water                                | 0.5     |
|                                      | 49.5    |

The refined oil is a distillate having an initial boiling point of about 350° F. and an end point of about 475° F. Although it is not necessary that these precise limits be maintained, it is important that a narrow cut be used of about this range: The so-called "W.W. 150" (water white kerosene), with a boiling range of about 373 to 504° F. evaporates too slowly, while oleum spirits, with a boiling range of about 300 to 425° F. evaporates too rapidly to give best results. The narrow boiling range of the refined oil is of particular importance in a "set" or solid emulsion of this type. It is also of particular importance that the oil be highly refined (treated with sulfuric acid for the removal of unsaturateds and other impurities) because I have found that un- 100

treated light petroleum distillates may be injurious to the skin.

The emulsifier is preferably ordinary starch, although equivalent emulsifiers may be used provided that they will give a stable emulsion as hereinafter described.

In preparing my finished product I melt the base stock with the refined oil and heat the mixture to a temperature of about 175 to 200° F. I then boil a 1% starch solution and make an oil-in-water emulsion in a colloid mill at a temperature above the melting point of the wax and below the boiling point of the water, usually at about 130 to 200° F. When the resulting emulsion cools, it sets to form a semi-hard, solidified emulsion which is extremely stable and which possesses entirely different structural properties from the ordinary liquid oil-in-water emulsions of the same concentrations. The product may be stored for an indefinite period of time without separation, and it may be easily handled and applied. Although my preferred formula calls for about 50% water, I may vary the formula 15 to 20% in either direction.

While I do not limit myself to any theory of operation I would like to point out a few features which I believe contribute toward the phenomenal success of this polish. The use of a narrow cut of an oil carrier results in the application of an even coat which on polishing is substantially free from oil. Since the polish is in the form of an aqueous emulsion, it spreads easily on any surface, wet or dry, and although it contains no abrasive material it has a pronounced cleaning effect, due apparently to its emulsified form and to the solvent power of the water contained as an external phase. Where the surface to be polished is excessively dirty, the wax may, of course, be preceded by an abrasive cleaner of the usual type. The polish is much easier to apply than solid wax polishes heretofore used and it yields a hard, durable, lustrous finish which is unexcelled.

While I have described a preferred embodiment of my invention it is understood that I do not limit myself to the details therein set forth except as defined by the following claims which are to be construed as broadly as the prior art will permit.

I claim:

1. A wax polish comprising a mixture of hard wax and a petrolatum wax incorporated in a light petroleum oil dispersed in a set aqueous emulsion.

2. A wax polish comprising a hard wax, and a petrolatum wax incorporated in a refined oil having a boiling range of about 350 to 475° F. dispersed in a solid aqueous emulsion.

3. A combination of claim 2 wherein the hard wax is carnauba wax.

4. A combination of claim 2 wherein the hard wax is Montan wax.

5. A wax polish comprising a hard wax, petrolatum wax, and petrolatum incorporated in a refined petroleum oil having a boiling range of about 350 to 475° F., said oil being dispersed in a set aqueous emulsion.

6. A wax polish comprising a set oil-in-water emulsion having about the following formula:

|                              | Percent |
|------------------------------|---------|
| Hard wax-petrolatum mixture  | 9       |
| Refined oil (350 to 475° F.) | 41      |
| Emulsifier                   | .5      |
| Water                        | 49.5    |

7. The method of making a wax polish for automobiles which comprises boiling about .5% starch in 49.5% water, and emulsifying therein a mixture of about 9% of a hard wax base with 41% of a refined light petroleum oil at a temperature below the boiling point of water and above the melting point of the wax base.

8. The method of making a solid wax polish 130 for automobiles which comprises incorporating a hard wax in a refined light oil carrier, emulsifying the same in a hot starch solution and allowing the emulsion to cool and solidify.

9. A wax polish comprising a hard wax-petrolatum mixture dissolved in a solvent having a boiling range of about 350-475° F., said wax and solvent being emulsified with a volume of water substantially equal to the volume of the solution, and an emulsifying agent for emulsifying said hard wax solution with said water.

10. The method of making a solid wax polish, which comprises forming a wax mixture consisting of about two parts of a hard wax of the class consisting of carnauba, Montan, candelilla 115 and japan wax with about one part of a plasticizing agent comprising a petrolatum wax, incorporating said wax mixture in a refined light oil carrier, emulsifying the light oil solution of wax in about an equal volume of water, and allowing 120 the emulsion to solidify.

11. A wax polish comprising a hard wax of the class consisting of japan wax, carnauba wax, Montan wax and candelilla wax admixed with a smaller volume of petrolatum wax, both waxes 125 being dissolved in a solvent having a boiling range of about 350-475° F., the solvent containing said wax being emulsified with a volume of water substantially equal to the volume of the wax solution, and an emulsifying agent for emulsifying the wax solution in the water.

MAURICE H. ARVESON.

135

140

145

150

## CERTIFICATE OF CORRECTION.

Patent No. 1,979,787.

November 6, 1934.

MAURICE H. ARVESON.

It is hereby certified that error appears in the printed specification of the above numbered patent requiring correction as follows: Page 1, line 27, for "petroleum" read petrolatum; and that the said Letters Patent should be read with this correction therein that the same may conform to the record of the case in the Patent Office.

Signed and sealed this 5th day of February, A. D. 1935.

Leslie Frazer

(Seal)

Acting Commissioner of Patents.